

3,351,541

ELECTRODEPOSITION OF THE  
PLATINUM METALS

Ernest H. Lyons, Jr., Marblehead, and Russell M. Dempsey, Hamilton, Mass., assignors to General Electric Company, a corporation of New York  
No Drawing. Filed Jan. 19, 1965, Ser. No. 426,634  
20 Claims. (Cl. 204—47)

Our invention relates to an improved process and plating bath for electrodepositing a bright, ductile platinum metal. Our invention is additionally directed to a process of obtaining bright, ductile platinum metal deposits on base metals.

A variety of processes are known for electrodepositing platinum metals to thicknesses of 0.001 inch or less. Roseleur's bath, an aqueous solution of a complex platinophosphate usually modified with suitable buffering and brightening agents, is representative of one type of bath. Another type of bath uses ammoniacal dinitrodiamminoplatinum as a source of the metal to be deposited. A third general type of bath is the alkali platinate bath usually stabilized by the addition of an alkaline oxalate.

Processes of the general types outlined above exhibit a number of well recognized disadvantages. Included in such disadvantages are (1) the difficulty in obtaining deposits of any appreciable thickness, (2) the hard, brittle character of the deposits, (3) the necessity of periodically replenishing the platinum metal within the plating bath, (4) the necessity of periodic polarity reversal, (5) low current efficiency, etc.

Atkinson in U.S. Patent 2,792,341, issued May 14, 1957, discloses a procedure for electrodepositing bright, ductile platinum. This teaching constitutes an apparent improvement over previously known platinum depositing processes, since it purports to overcome the difficulties in obtaining relatively thick, ductile platinum deposits and also to overcome the necessity of periodically replenishing the platinum content of the bath. One of the distinct disadvantages of the Atkinson process is the requirement that hydrochloric acid be employed in a minimum concentration of approximately 5 moles, preferably 6.5 moles, and at temperatures above approximately 110° F. and preferably above 150° F. As recognized in the patent, the high acid concentration precludes direct electrodeposition on a base metal such as iron, copper, nickel, zinc, silver, etc. Other patent-recognized disadvantages include the tendency of tungsten and molybdenum to react with hydrochloric acid to form insoluble acid deposits. Further, the difficulty, due to evaporation, of maintaining concentrated hydrochloric acid at high temperatures was affirmed by Atkinson in 1959 (R. H. Atkinson, Vol. 7, Transactions of the Institute of Metal Finishing, p. 36) and in 1963 (R. H. Atkinson, Modern Electroplating, p. 316).

It is an object of our invention to provide an improved process and plating bath for electrodepositing bright, ductile platinum metal.

It is another object of the invention to deposit bright, ductile platinum metal without the use of concentrated acids.

It is a further object to provide a process for electrodepositing bright, ductile platinum metal at reduced temperatures.

These and other objects of our invention are accomplished by employing an aqueous plating bath containing in solution at least 100 grams/liter (g./l.) of a lithium or alkaline earth metal halide and from 1 to 50 g./l. of a platinum metal in quadrivalent form, preferably in the form of platinum metal hexahalide anions. Electrodeposition of the platiump metal is effected at a cathode,

which may be formed of a base metal, while the anode is preferably formed of the platinum metal, whereby the bath may be continuously replenished. Deposition is conducted at current densities ranging from 10 to 200 milliamperes per square centimeter and at temperatures ranging from 30° C. to 110° C.

The term "platinum metal" as herein employed includes Group VIII metals of the light and heavy platinum triads, excepting osmium and iridium. These metals are ruthenium, rhodium, palladium, and platinum. The term "halide" as herein employed includes Group VIIA anions with the exception of fluoride. The included halides consist of chlorides, bromides, and iodides. Generally, chlorides are preferred because of their greater availability and lesser cost.

The platinum metal is present in the bath in quadrivalent form with small amounts of divalent platinum metal also usually being present. The ratio of quadrivalent platinum metal to divalent platinum metal should be greater than 20 to 1. A preferred platinum metal compound for use in our plating bath is chloroplatinic acid. Other exemplary additives include chloropalladic acid as well as chlorides of ruthenium and rhodium. Platinum metal halides may be employed individually or as mixtures in any proportion. Platinum metals may also be added to the bath in the form of sodium, lithium, or alkaline earth platinum metal halides such as, for example, sodium chloroplatinate, lithium chloroplatinate, alkaline earth chloroplatinates, etc. as well as analogs thereof. Other useful platinum metal additives include hydrated platinum metal oxides such as hydrated platinic oxide for example.

The bath electrolyte is a lithium or alkaline earth metal halide having a solubility of at least 100 g./l. Lithium halides are generally preferred electrolytes because of their relatively higher solubilities. Lithium chloride is a preferred electrolyte. Exemplary suitable alkaline earth metal halides include magnesium, calcium, strontium, and barium chloride as well as analogs thereof. If desired, the bath may be saturated with the electrolyte.

It is contemplated to use either soluble platinum metal anodes or insoluble anodes made from material inert to the action of the electrolyte as, for example, tantalum. When a platinum metal anode is employed, the anode will enter the bath solution at the rate of metal deposition, rendering metal replenishment unnecessary. When an inert anode is employed, the platinum metal constituent of the bath may be replenished by any conventional procedure.

A conventional electrode may be employed as a cathode. Whereas acid and other highly corrosive electroplating baths are limited to the use of noble metal electrodes, our invention is practicable with either a noble or base metal cathode. In other words, our invention may be used to electroplate metal articles formed from such materials as palladium, gold, silver, nickel, copper, etc., irrespective of whether such articles are attacked by strong reagents, such as hydrochloric acid, or not.

Plating is conducted at temperatures ranging from 30° C. to 110° C. and at cathode current densities of from 10 to 200 ma./cm.<sup>2</sup>. The current density is calculated on the basis of the immersed cathode surface area facing the anode, as is conventional practice. Plating may be conducted in any convenient, conventional cell configuration. Since lithium and alkaline earth metal halides do not exhibit the high degree of volatility of hydrochloric acid and since operating temperatures may be substantially lower than those employed in corresponding hydrochloric acid plating baths, only nominal bath maintenance is required.

Plating may be continued for any time duration necessary to build up a platinum metal deposit of the desired

thickness. While economic considerations generally dictate thin platinum metal coatings, the process is not limited to the deposition of thin coatings. Unlike conventional platinum metal plating processes, our process may be employed to generate coatings in excess of 1 mil in thickness without resort to ancillary manipulations such as polishing, current reversals, etc.

As is well recognized in the art, the bath should be maintained free of contaminants which will adversely influence the plating process, as for example, strong oxidizing agents, strong reducing agents, undesirable base metals which may co-deposit with the platinum metals, etc. Potassium, ammonium, cesium, rubidium, etc., ions should be substantially absent from the bath because of the well-known tendency of these materials to cause the precipitation of platinum metals as insoluble salts of the hexahalogeno-platinic acid. Impurities of the type normally associated with commercial grades of platinum metals are not, however, considered objectionable to the practice of the invention.

While our process is described in terms of the best mode contemplated for its performance, numerous variations will be readily apparent to those skilled in the art. The process constitutes an improvement over the process of Atkinson in substituting lithium or alkaline earth metal halides for hydrochloric acid, however, the invention could, if desired, be practiced using a mixture of hydrochloric acid and metal halides. In such instance, the adverse effects of hydrochloric acid are proportionately decreased.

The following examples are illustrative of the practice of our invention and are not for purposes of limitation:

*Example 1*

A plating bath is formed consisting essentially of 400 g./l. lithium chloride and 9 g./l. chloroplatinic acid. The bath is maintained at a temperature of 50° C. A massive platinum anode is immersed in the bath along with a copper cathode in the form of a thin strip. A current of 62.5 milliamperes per square centimeter is maintained between the electrodes for a period of approximately 10 minutes.

Upon removal from the bath the copper strip is noted to be coated with a bright silver-colored deposit. The strip is bent repeatedly without any detectable scaling of the coating and without breaking.

*Example 2*

The procedure of Example 1 is repeated, except that plating is continued for 30 minutes. Upon removal from the bath, the copper strip is noted to be coated with a bright, silver-colored deposit. The thickness of the deposit is visible to the eye and therefore noted to be in excess of 1 mil. The strip is bent repeatedly without breaking or scaling.

*Example 3*

The procedure of Example 1 is repeated substituting a palladium cathode in strip form for the copper cathode. Upon removal from the bath, a barely discernible line of junction between the platinum deposit and the palladium strip is detected. The platinum coating is noted to be of a brightness at least equal to that of the palladium strip. Upon repeated flexing, neither scaling nor breaking is noted.

*Example 4*

The procedure of Example 1 is repeated substituting a nickel strip for the copper cathode. The results achieved substantially duplicate the results obtained using a copper cathode.

*Example 5*

A plating bath is prepared by adding slightly more calcium chloride than is required to form a saturated solution at 80° C. Fifty grams/liter chloropalladic acid is added. The bath is maintained at 80° C.

A palladium metal anode is immersed in the bath along with a copper cathode. A current density of 40 ma./cm.<sup>2</sup> is maintained for a period of 15 minutes.

Upon removal from the bath, the copper strip is noted to be coated with a bright, silver-colored deposit. The strip is bent repeatedly without any detectable scaling of the coating and without breaking.

What we claim as new and desire to secure by Letters Patent of the United States is:

1. A process of electroplating a platinum metal comprising
  - preparing an aqueous plating bath containing in solution at least 100 grams/liter of an electrolyte chosen from the group consisting of lithium halide and alkaline earth metal halide and from 1 to 50 grams/liter of a platinum metal in quadrivalent form,
  - maintaining the aqueous plating bath at a temperature of from 30° C. to 110° C.,
  - immersing an anode and a cathode in the plating bath, and
  - maintaining a cathode current density of from 10 to 200 milliamperes per square centimeter.
2. A process according to claim 1 in which said electrolyte is lithium chloride.
3. A process according to claim 1 in which said electrolyte is calcium chloride.
4. A process according to claim 1 in which the platinum metal is platinum.
5. A process according to claim 1 in which the platinum metal is palladium.
6. A process according to claim 1 in which the platinum metal is present in the bath in the form of chloroplatinic acid.
7. A process according to claim 1 in which the platinum metal is present in the bath in the form of chloropalladic acid.
8. A process according to claim 1 in which the anode is platinum.
9. A process according to claim 1 in which the anode is palladium.
10. A process according to claim 1 in which the cathode is a noble metal.
11. A process according to claim 1 in which the cathode is a base metal.
12. A process of electroplating a platinum metal comprising
  - preparing an aqueous plating bath containing in solution at least 100 grams/liter of an electrolyte chosen from the group consisting of lithium chloride and alkaline earth metal chloride and from 1 to 50 grams/liter of a platinum metal in the form of divalent platinum metal hexachloride anions,
  - maintaining the aqueous plating bath at a temperature of from 30° C. to 110° C.,
  - immersing an anode and a cathode in the plating bath, and
  - maintaining a current density between the anode and cathode of from 10 to 200 milliamperes per square centimeter.
13. A process according to claim 12 in which the platinum metal is present in the bath in the form of chloroplatinic acid and the anode is platinum.
14. A process according to claim 12 in which the platinum metal is present in the bath in the form of chloropalladic acid and the anode is palladium.
15. A process according to claim 12 in which the cathode is a base metal.
16. An aqueous plating bath containing in solution at least 100 grams/liter of an electrolyte chosen from the group consisting of lithium halide and alkaline earth metal halide and from 1 to 50 grams/liter of platinum metal in quadrivalent form.
17. A plating bath according to claim 16 in which the platinum metal is present in the form of divalent platinum metal hexahalide anions.

18. A plating bath according to claim 17 in which the platinum metal is present in the bath in the form of chloroplatinic acid.

19. An aqueous plating bath containing in solution at least 100 grams/liter of an electrolyte chosen from the group consisting of lithium chloride and alkaline earth metal chloride and from 1 to 50 grams/liter of a platinum metal in the form of divalent platinum metal hexachloride anions.

20. An aqueous plating bath according to claim 19 in which the platinum metal is platinum.

## References Cited

## UNITED STATES PATENTS

|           |         |              |          |
|-----------|---------|--------------|----------|
| 2,457,021 | 12/1948 | Wise et al.  | 204-47   |
| 2,470,033 | 5/1949  | Hensel       | 204-47 X |
| 2,720,494 | 10/1955 | Suter et al. | 204-47 X |
| 2,792,341 | 5/1957  | Atkinson     | 204-47   |

JOHN H. MACK, Primary Examiner.

10 G. KAPLAN, Assistant Examiner.